

## UNITED STATES PATENT OFFICE

CHARLES HUGH ROBERTS GOWER, OF LONDON, ENGLAND, ASSIGNOR TO ALUMINUM  
COLORS INCORPORATED, OF INDIANAPOLIS, INDIANA, A CORPORATION OF INDIANA

## ANODIC COATING OF ALUMINUM

No Drawing. Application filed October 29, 1931, Serial No. 571,945, and in Great Britain October 20, 1927.

This invention relates to anodic coating of aluminum; and it comprises an article of aluminum or aluminum alloy carrying a coating of substantial thickness having the general characteristics of a coating produced by making such an article an anode at low voltages in sulfuric acid of low concentration approximating 15 to 35 per cent by weight, this coating containing  $\text{Al}_2\text{O}_3$ ,  $\text{SO}_3$  and  $\text{H}_2\text{O}$  in combination, being laminar with a flint-like underlayer and a somewhat softer outer layer, being insoluble, resistant to wear and abrasion, absorptive, porous and capable of being buffed and polished; and it also includes a process of coating aluminum articles which comprises immersing such articles in a bath of sulfuric acid of a low concentration approximating 15 to 35 per cent by weight and passing an electric current at low voltages from such articles to other electrodes in said bath, this treatment being followed by various other operations such as rinsing, dyeing, buffing, polishing, oiling, pigmenting, etc; all as more fully hereinafter set forth and as claimed.

The present application is a continuation in part of my copending application Serial No. 253,790, filed February 11, 1928, and comprises certain extensions of the methods therein described as well as improvements in the articles produced. In my earlier application I described a process of coating aluminum articles by making the same anodes at low voltages in a bath of sulfuric acid of a concentration ranging from  $1\frac{1}{2}$  to 2 pounds per gallon or approximately 15 to 20 per cent of  $\text{H}_2\text{SO}_4$  by weight.

I have now found that the upper limit of the concentration range can be extended up to 35 per cent sulfuric acid with some advantages, an optimum value apparently lying in the neighborhood of about 25 per cent. At concentrations below 15 per cent there is a decided increase in cost due to a higher current consumption. A different type of coating appears to be formed at these lower concentrations which is not laminar, a feature which is a characteristic of my coatings. At concentrations above 35 per cent the coatings formed are not as adherent. They usually

chip and craze. Consequently there is a rather narrow range of acid concentration over which the most advantageous coatings are obtained.

The coatings obtained over this particular acid range are characterized by their laminar structure which consists in a flint-like underlayer and a somewhat softer outer layer, the latter still being sufficiently hard to withstand buffing, abrasion, etc. Using the so-called microcharacter scratch test for hardness, with a standard 3 gram load, one specimen, coated in a 25 per cent bath, was found to have a surface hardness of 140. The hardness next to the metal was found to be 5000. This is in comparison with glass and with chromium having hardnesses of 2000 and 3100, respectively.

In spite of their hardness my coatings are firmly coherent to the underlying metal which can be bent to a considerable extent without damaging the coating. Although hair line cracks are likely to appear this has been found not to impair the resistance to corrosion.

My coatings are minutely pervious, the pores being sub-microscopic and having a volume amounting to about 25 per cent of the total volume of the coating. These pores are capable of absorbing and adsorbing various materials such as dyes, pigments, oils, paints, etc. A treatment with such materials greatly improves the corrosion resistance by plugging the pores and making them impervious. The  $\text{SO}_3$  content ranges from about 12 to 16 per cent by weight and  $\text{SO}_3$  appears to be a necessary component of my coatings. My coatings are insoluble in water and resistant to the acid of the coating bath.

The thickness of my coatings and their laminar structure distinguish them clearly from the prior art, in which generally films were obtained of no substantial thickness and providing but slight protection from corrosion. Satisfactory coatings for my purposes range in thickness from about 0.0002 to 0.001 inch. In order to obtain coatings 0.0002 inch thick, a treatment in the sulfuric acid bath of only 10 minutes, at about 12 volts, is required. The thicker films require

a time of treatment ranging up to 45 minutes or an hour. Longer treatments do no harm but the thickness of the film is not substantially increased after an hour.

- 8 The voltages suitable for my process range from about 6 up to 20 volts. So-called "addition agents" can be added to the bath if desired. Ordinary room temperatures may be used, that is temperatures ranging from 10 about 60° to 100° F. Practically any type of aluminum alloy is suitable, whether rolled or cast. The alloys should contain at least 15 85 per cent of aluminum. Some of the alloys produce colored or tinted coatings, but the usual color of the coating produced on substantially pure aluminum is pearlish cloudy white. Duralumin produces a gray coating, this color also resulting with alloys containing silicon or tin.
- 20 In a specific embodiment of my invention I may take an article of pure rolled or cast aluminum and polish the same. The article should then be carefully cleaned by being immersed in a solvent for grease and thereafter rinsing. Castings should be cleaned mechanically with an abrasive powder and brush to assure that all holes and cavities are free from dirt, prior to cleaning in the grease solvent. The cleaned article is then connected with 30 a source of electrical potential and made the anode in a bath comprising an aqueous solution of sulfuric acid of 25 per cent strength by weight, care being taken that the object is not put into the bath unless the electric current is on. The cathode may be of carbon or lead. The object may be suspended in the bath in electrical connection by thick aluminum wires or aluminum clamps, care being taken that the length of connecting 40 conductor in the solution is as short as possible; or it may be suspended by wires of metals not attacked by the bath. In the case of big sheets, castings or objects in which a coating of absolutely uniform appearance is 45 not essential the object may be partially immersed and treated and then inverted so that the remainder of the surface may be similarly treated, the electrical connections in each case being made outside the bath. The voltage 50 across the bath may preferably be about 6 volts. With this voltage, when the object is first immersed the current rises to about 10 amperes per square foot which rapidly falls to a steady current of about 2 amperes 55 per square foot. This procedure will give a satisfactory coating in about 25 minutes. The bath should be stirred or agitated before and during use. The bath should be brought back to strength from time to time by the 60 addition of the correct amount of sulfuric acid.

After the anodic treatment, the article should be removed from the sulfuric acid bath and washed with water. It may then 65 be dyed or, after drying, the pores may be

plugged with oil, pigments, paint, lacquer and the like. Buffing imparts a highly glossy finish and the usual grease buffering compounds also fill the pores.

What I claim is:

- 70 1. In the anodic coating of aluminum and aluminum alloy articles, the process which comprises treating such articles anodically with low working voltages in a bath of sulfuric acid having a low concentration of 75 about 25 per cent by weight.
2. In the anodic coating of aluminum and aluminum alloy articles, the process which comprises treating such articles anodically 80 with low working voltages in a bath of sulfuric acid having a concentration ranging from about 15 to 20 per cent by weight.
3. In the anodic coating of aluminum and aluminum alloy articles, the process which 85 comprises treating such articles anodically with low working voltages in a bath of sulfuric acid having a concentration ranging from more than 20 to 35 per cent by weight.
4. In the anodic coating of aluminum and aluminum alloy articles, the process comprising 90 passing current from such articles to other electrodes in an electrolytic bath having a concentration of about 15 to 20 per cent sulfuric acid and with voltages ranging from 6 to 20 volts.
5. In the anodic coating of aluminum and aluminum alloy articles, the process comprising 95 passing current from such articles to other electrodes in an electrolytic bath having a concentration of more than 20 to 35 per cent 100 sulfuric acid and with voltages ranging from 6 to 20 volts.
6. In the anodic coating of aluminum and aluminum alloy articles, the process which 105 comprises anodically coating such articles in a bath of sulfuric acid having a concentration ranging from about 15 to 20 per cent by weight and finally plugging the pores of the coating so formed.
7. In the anodic coating of aluminum and 110 aluminum alloy articles, the process which comprises anodically coating such articles in a bath of sulfuric acid having a concentration ranging from more than 20 to 35 per cent by weight and finally plugging the pores of the 115 coating so formed.
8. In the anodic coating of aluminum and aluminum alloy articles, the process which 120 comprises anodically coating such articles in a bath of sulfuric acid having a concentration ranging from about 15 to 20 per cent by weight and finally filling the pores of said coating with oil.
9. In the anodic coating of aluminum and 125 aluminum alloy articles, the process which comprises anodically coating such articles in a bath of sulfuric acid having a concentration ranging from more than 20 to 35 per cent by weight and finally filling the pores of said 130 coating with oil.

10. In the anodic coating of aluminum and aluminum alloy articles, the process which comprises anodically coating such articles in a bath of sulfuric acid having a concentration ranging from about 15 to 20 per cent by weight and finally buffing said coating.
11. In the anodic coating of aluminum and aluminum alloy articles, the process which comprises anodically coating such articles in a bath of sulfuric acid having a concentration ranging from more than 20 to 35 per cent by weight and finally buffing said coating.
- 10 12. As a new article, a body of aluminum or aluminum alloy carrying a coating of substantial thickness having the general characteristics of one produced by making such an article an anode at low voltages in a sulfuric acid bath of low concentration of 15 to 20 per cent by weight, this coating containing  $Al_2O_3$ ,  $SO_3$  and  $H_2O$  in combination, being laminar with a flint-like under layer and a somewhat softened outer layer, being insoluble, resistant to wear and abrasion, absorptive and adsorptive, porous and capable of being buffed.
- 15 13. As a new article, a body of aluminum or aluminum alloy carrying a coating of substantial thickness having the general characteristics of one produced by making such an article an anode at low voltages in a sulfuric acid bath of low concentration of more than 20 to 35 per cent by weight, this coating containing  $Al_2O_3$ ,  $SO_3$  and  $H_2O$  in combination, being laminar with a flint-like under layer and a somewhat softened outer layer, being insoluble, resistant to wear and abrasion, absorptive and adsorptive, porous and capable of being buffed.
- 20 14. The article of claim 12 in which the pores of said coating are plugged, thereby rendering the said coating more resistant to corrosion.
- 25 15. The article of claim 13 in which the pores of said coating are plugged, thereby rendering the said coating more resistant to corrosion.
- 30 16. The article of claim 12 in which the pores of said coating are filled with oil, thereby rendering the said coating more resistant to corrosion.
- 35 17. The article of claim 13 in which the pores of said coating are filled with oil, thereby rendering the said coating more resistant to corrosion.
- 40 18. The article of claim 12 in which the said coating has been finished by buffing.
- 45 19. The article of claim 13 in which the said coating has been finished by buffing.
- 50 In testimony whereof I have hereunto, affixed my signature.
- 55 CHARLES HUGH ROBERTS GOWER.